

May 12, 1936.

H. W. NIEMAN

2,040,442

METHOD OF TREATING SHEET METAL

Filed Nov. 30, 1932

FIG. 1.



FIG. 2.



FIG. 3.



Inventor

Henry W. Nieman,

By R. S. C. Dougherty.  
Attorney

## UNITED STATES PATENT OFFICE

2,040,442

## METHOD OF TREATING SHEET METAL

Henry W. Nieman, Bethlehem, Pa., assignor to  
Bethlehem Steel Company, a corporation of  
Pennsylvania

Application November 30, 1932, Serial No. 644,972

12 Claims. (Cl. 153—54)

The present invention relates to methods of conditioning mild steel sheets, strips, and analogous thin flat articles for subsequent fabrication into articles of manufacture.

A large quantity of steel sheets or strips having a carbon composition in the neighborhood of  $\frac{1}{16}\%$  are rolled in the manufacture of tinplate, automobile sheets and the like, the reduction to final gauge being made either by hot or cold rolling. In either case the metal as it leaves the rolls is in a hard and unworkable condition and usually must be given an anneal. This renders the metal soft and ductile but at the same time introduces an undesirable quality, a tendency to "flute" or form "stretcher strains" upon subsequent fabrication.

Fluting and stretcher straining of annealed low-carbon sheet material may be designated its peculiar and very undesirable property of yielding locally instead of over a broad area when deformed beyond its yield point. A mild steel sheet which bends sharply at one point instead of curving uniformly over a broader area when subjected to flexing forces is said to "flute." A mild steel sheet, the surface of which apparently cracks when the sheet is subjected to a tension beyond its elastic limit, is said to "stretcher strain".

When a sheet of such material is elongated in a testing machine, no permanent set takes place until the very definite yield point is reached. Then a series of apparent cracks develops as the elongation continues, and these cracks, which are known as "stretcher strains", broaden out until they finally meet and cover the entire area, which then has a matte appearance quite different from the originally shiny appearance of the sheet. As the elongation is continued from this point on, the tension increases gradually until the specimen necks out, and breakage finally results. If the test is halted when the stretcher strains have covered only a portion of the surface, it is found that the material, as measured in a strained area, is thinner than the original sheet. The phenomena of stretcher straining is particularly observed in the fabrication of automobile bodies and similar objects where the stretching of certain parts of the sheet by the dies is sufficient to cause "stretcher strains" but not sufficient to cause these to coalesce into a relatively smooth surface. The resulting pattern is, of course, highly undesirable.

Various methods have heretofore been employed for the removal of the tendency to strain and flute from a mild steel annealed sheet. Thus, it

has been common to give the sheet, after annealing, a light cold rolling or "planishing." While this method of eliminating the tendency of the sheet to flute upon fabrication is, in most instances when utilized, capable of producing the desired results, it is not always a practical or desirable method in that the cold rolling operation must be carried out very carefully to avoid warping the sheet or hardening it unduly and also by reason of the fact that a new surface is imparted to the sheet by the rolls, which is often undesirable, for instance where the sheet has been previously tin-coated.

Again, it is known that mild steel annealed sheets may have their qualities improved, insofar as fluting and stretcher straining are concerned, by passing them through roller levelers. It has been found, however, that the use of a roller leveler is not possible in connection with certain strips or sheets because of the very pronounced tendency of the sheets to flute or wrinkle in the leveler, and, moreover, with other steels which do not actually wrinkle there frequently are formed thereon multitudes of fine parallel lines. These may be too fine for measurement but still deface the surface.

I have discovered that the tendency of mild steel annealed sheets to flute or to form stretcher strains, during fabrication, may be completely eliminated or removed by subjecting such sheets after annealing to a special hot working process, the nature of which will hereinafter be set forth in detail.

I have discovered that sheet steel, even though it has a pronounced tendency to flute or form stretcher strains at ordinary room temperatures, can be bent or stretched smoothly when heated to a point above a certain definite critical temperature which is generally between 700° and 750° F. If an annealed sheet of tin plate gauge (and the average tin plate gauge is in the neighborhood of 12/1000 of an inch) is heated to this temperature and bent over a roller of three inches in diameter first in one direction and then in the other, while the sheet is cooling, it will be found that when cold the sheet will no longer flute in any direction and will show only extremely shallow stretcher strains when stretched. As few as four bending operations accomplish this result although it is generally desirable to employ more. The qualities of the metal will even be considerably improved by two flexures of the metal at this temperature, the flexures being in opposite directions.

The ability of annealed sheet steel to bend or

stretch smoothly when heated to a certain definite temperature makes it possible to treat such material in a further and different manner for the elimination of its tendency to flute or form stretcher strains in subsequent fabrication. Thus, if the metal is stretched while in the heated condition to a limited extent, say 1% or 2% of its total length, it is found that the qualities of the metal are greatly improved; that is, it is found that when the metal, after it is cooled, is submitted to fabrication, it will work smoothly and has no tendency to flute or to form stretcher strains.

Various types of apparatus are suitable for carrying on the treatment of the metal in accordance with the methods above outlined, and my invention is in no wise limited in its broader aspect to any particular apparatus. In the accompanying drawing I illustrate three forms of apparatus which I have found entirely suitable in practice, but one skilled in the art will readily appreciate that in carrying out the method under varying circumstances the actual apparatus used may be very widely varied in the design and arrangement of its component elements without departure from the invention.

In the drawing:

Figure 1 shows diagrammatically apparatus for the undulation or flexure of a traveling sheet or strip when in heated condition;

Figure 2 illustrates, also diagrammatically, a suitable apparatus for subjecting a sheet or strip to a stretching operation while in heated condition; and

Figure 3 is a diagrammatic showing of apparatus for the manufacture of tinned sheets, which apparatus includes means for reconditioning the sheets after they have been subjected to the action of the tin pot.

The apparatus disclosed in Figure 1 of the drawing comprises essentially a reel 10 upon which a strip or sheet of annealed mild steel is wound, 11 a furnace, 12-12 a series of rollers, and 13 a second reel or drum upon which the sheet is wound after it passes through furnace 11 and past the rollers 12. The sheet metal on drum 10 may be in the annealed state or may be in its hardened condition as it comes from the rolling mill. If the metal is already annealed, the heating furnace 11 will comprise in effect a reheating furnace while, if the sheet on the drum 10 has not been annealed, the furnace 11 may comprise a continuous heating furnace of the type satisfactory for carrying on the annealing operation. In carrying out the process, the metal is passed through the furnace 11 at such speed that it is brought to a temperature of approximately 700°, preferably somewhat higher, and then passed directly over the rollers 12, at which point it is given four flexures, two in one direction and two in the other. The metal gradually cools during this undulatory treatment and leaves the final roller 12 at a comparatively low temperature.

Sheet metal treated by this method is not only smooth working and pliable but suffers practically no impairment of its physical properties by reason of the treatment. It may even show improvement. The exceedingly mild mechanical treatment it receives does not in any way injure the surface.

In Figure 2 of the drawing, an apparatus for stretching the metal while in the heated condition is shown.

Here the sheet is pulled from the drum 20,

which is provided with a brake to furnish back tension, over the idler cylinder 21 and through a pot of molten salts 22 which furnishes the heat, over the rolls 23 and 24 and on to the drum 25, which is driven from a suitable source of power. The rolls 23 and 24 are geared together with a one-to-one ratio, the gears being indicated at 23' and 24', respectively, but the roll 24 is of slightly greater diameter than the roll 23. As a result of this arrangement, the sheet is stretched as it bridges the gap between rolls 23 and 24 by the exact amount of the difference in surface speeds of these rolls. It has been found that an arrangement such as just described, by means of which a strip passing through the apparatus is lengthened about 1½%, will impart a very satisfactory quality to the strip without injuring its surface or physical properties.

Sheet steel that has been treated according to the above method or by any other method for the elimination of the tendency to flute or form stretcher strains will tend to age, that is, will tend to slowly return to its initial unsatisfactory condition. This ageing usually progresses so slowly that it is not an important factor, but, on the other hand, if the metal is subjected to a higher temperature even for a very short time, the ageing proceeds with great rapidity, and the metal may be seriously impaired.

After passing through a tin pot, for instance, the temperature of which is in the neighborhood of 600° F., it will be found that the metal, even if previously treated by one of the above methods or by roller leveling or by cold rolling to remove the tendency to flute or form stretcher strains, will partially revert to its original annealed condition. It has been found that this ageing or return to its original condition can be prevented by passing the strip over a series of rollers immediately after it emerges from the molten tin, with the result that, when cold, it will still work smoothly. As the temperature of the tin is about 600° F., it may seem that this is in contradiction to the statement made at the beginning that a temperature of about 700° F. is necessary for the first bending operation. In this case, however, we are dealing with material that has already been treated so that, before it enters the tin pot, it works smoothly.

The results may be stated more generally as follows: Low-carbon steel sheets after annealing are subject to stretcher strains and fluting at room temperatures when they are fabricated, but these effects may be eliminated by either undulating or stretching, commencing at a temperature above 700° in accordance with either of the methods set forth above. In the event, however, that a sheet or strip has been subjected to such a hot stretching or hot undulating process or any other process which has placed the material in suitable condition for fabrication, that is, any smooth working condition, and is thereafter subjected to the application of heat below 700° F. in temperature, it is possible to prevent a reversion of the metal to its original state by bending or undulating the same at a temperature below 700° F. This fact makes it possible to first stretch or undulate sheet metal, commencing at a temperature above 700° to eliminate its tendency to flute or form stretcher strains, to thereafter pass the metal through a tin pot having a temperature in the neighborhood of 600°, and to subsequently prevent reversion of the newly heated metal to its original state by undulating the same over a series of rollers immediately after it issues from

the tin pot. A suitable apparatus for carrying out this method is diagrammatically shown in Fig. 3 of the drawing.

Here a cold rolling mill is indicated at 30, a continuous annealing furnace at 31, a tin pot at 32, and a series of rollers, for undulating the sheet after emergence from the tin pot, at 33. Rolls 34 may be utilized to give the cold rolled and annealed sheets a "pinch pass" to partially, at least, condition them before they enter the tin pot. Instead of rolls 34, however, an undulating machine, such as disclosed in Figure 1, may be substituted, the object being to completely condition the sheets prior to subjecting them to the tinning operation. As has been before pointed out, passage of the sheet material through the tin pot effects its very rapid "ageing" which reduces the effect of any previous treatment to remove the tendency to flute or stretcher strain. The undulation of the tinned sheet while it still has a temperature of approximately 600° F. reconditions the same very satisfactorily, however, and the resulting product is a tinned sheet with good deep drawing properties and without tendency to flute or form stretcher strains.

No satisfactory explanation has been advanced to explain the occurrence of stretcher strains in low carbon, whereas high-carbon steel, alloy steel, and other metals are, so far as I am aware, free from them. Nor is it understood why they do not occur at higher temperatures. A probable explanation is that at the temperatures found necessary for hot undulating of annealed sheets, about 725° F., the slippage due to working the material will follow the grain boundaries almost exclusively so that any working applied to the metal at this temperature will be working the boundary material and not the material of the grains themselves, so that a substantial amount of amorphous material will accumulate between the grains. If mild working is then continued as the metal cools, amorphous material will not only be prevented from reverting to its crystalline state, but more will form, and when cold the grains will all be enclosed in an envelope of such material.

The condition where the grain boundaries of a fine grain steel are strained and rendered more or less amorphous, with the grains themselves unstrained, is an ideal one for subsequent working as it will bend or stretch without fluting or the formation of stretcher strains while at the same time the strength and ductility are unimpaired. It will be understood, however, that the theory stated above is difficult if not impossible to demonstrate conclusively and is offered only as a possible explanation of the necessity, which has been clearly demonstrated, of following the process outlined to achieve the desired results.

Where the sheet material is treated by stretching, it may be found desirable to perform the actual elongation in a series of operations rather than in a single one. The first stretching operation is preferably carried out while the section of the sheet under tension has a temperature of about 750° F. There is no upper limit of temperature, but higher temperatures should be avoided as the metal is harder to handle and also oxidizes more freely. The second stretching operation may be carried out with the metal at a temperature of approximately 600° F., the third operation at 500° F., the fourth operation at 400° F., and the fifth at 300° F. At each operation the metal is elongated approximately 1% of its length. The steps may be performed by one passage of

the sheet successively through four rotary stretching machines. Obviously the temperatures advised above need not be exactly obtained in practice, and also the number of stretching operations may be varied as found desirable. A sheet 5 treated in this manner, however, is put into excellent condition for further fabrication.

I have also found that tinned sheets, as well as untinned sheets, may have their properties improved by hot stretching, and hence I contemplate utilizing, if desired, stretching machines in lieu of undulating machines in treating the sheet metal after it emerges from the tin pot. Treating the metal by working the same at elevated temperatures to remove the tendency to flute need 10 not be done where it is possible to fabricate the sheets, etc., directly into finished articles at such temperatures. Thus, it is quite possible to make certain articles (such, for instance, as sheet metal pipes) without fluting the metal, provided it is 15 maintained at a sufficiently high temperature during fabrication, preferably at a minimum temperature of 700° F.

My discovery may be taken advantage of also in another way. Thus, by heating to a temperature of 700° F., or above, a mild steel annealed sheet or strip coiled upon a drum or the like, the metal may be unwound from the drum without without fluting, whereas if the same metal were unwound at ordinary temperature from the coil, 30 it might be greatly damaged by the formation of flutes. To one skilled in the art, it will be apparent also that the process of treating or fabricating the metal while hot may be helpful in connection with many other operations. 35

Naturally the specific means employed to carry out the process may be varied considerably in adapting the invention to the treatment of sheets of various thicknesses and compositions, without departure from the spirit of the invention. 40

Having thus described my invention, what I claim as new and desire to secure by Letters Patent is:

1. The method of producing a mild steel sheet with tinned surfaces and good drawing properties, substantially free from tendency to flute or stretcher strain, which comprises cold rolling the sheet to gauge, annealing the same, treating the sheet to lessen its tendency to flute or stretcher strain, passing the same through a tin pot, immediately thereafter, while still at an elevated temperature, submitting the same to deformation and then cooling the same with sufficient promptness to avoid substantial reversion to a fluting or stretcher straining condition. 45

2. The method of producing a mild steel sheet with tinned surfaces and good drawing properties, substantially free from tendency to flute or stretcher strain, which comprises cold rolling the sheet to gauge, annealing the same, treating the sheet to lessen its tendency to flute or stretcher strain, passing the same through a tin pot, immediately thereafter, while still at an elevated temperature, reversely flexing the same and then cooling the same with sufficient promptness to avoid substantial reversion to a fluting or stretcher straining condition. 60

3. The method of fabricating mild steel sheet metal which comprises plastically forming the same into manufactured articles while maintaining the temperature of the metal in the range above and adjacent to the minimum temperature at which the metal in its annealed state is free from the tendency to flute and stretcher strain. 75

4. The method of producing mild steel tinned sheets or the like which includes stretching the sheet immediately after its emergence from the tin pot and before it has cooled and then cooling the same with sufficient promptness to avoid substantial reversion to a fluting or stretcher straining condition.
5. The method of eliminating the tendency of sheets and the like to flute or stretcher strain in forming operations which comprises submitting the same to deformation while at a temperature in the range above and adjacent to the minimum temperature at which the metal in its annealed state is free from the tendency to flute and stretcher strain and then cooling the same with sufficient promptness to avoid substantial reversion to a fluting or stretcher straining condition.
6. The method of eliminating the tendency of sheets and the like to flute or stretcher strain in forming operations which comprises oppositely flexing the same while at a temperature in the range above and adjacent to the minimum temperature at which the metal in its annealed state is free from the tendency to flute and then cooling the same with sufficient promptness to avoid substantial reversion to a fluting or stretcher straining condition.
7. The method of uncoiling a coiled strip of mild steel which tends to flute when straightened at ordinary temperatures comprising the step of uncoiling the strip while within the temperature range of about 700° F. to red heat.
8. The method of eliminating the tendency of sheets and the like to flute or stretcher strain which comprises submitting the same to deformation at elevated temperatures and to further deformation during cooling.
9. The method of eliminating the tendency of sheets and the like to flute or stretcher strain which comprises submitting the same to deformation while at a temperature of 700° F. or above and to further deformation at lower temperatures.
10. The method of eliminating the tendency of sheets and the like to flute or stretcher strain which comprises oppositely flexing the same at elevated temperatures and to further flexing while cooling.
11. The method of producing a mild steel sheet with tinned surfaces and good drawing properties, substantially free from tendency to flute or stretcher strain, which comprises cold rolling the sheet to gauge, annealing the same, treating the sheet to lessen its tendency to flute or stretcher strain, passing the same through a tin pot, and immediately thereafter, while still at an elevated temperature, submitting the same to strain and submitting the same to further deformation while cooling.
12. The method of producing a mild steel sheet with tinned surfaces and good drawing properties, substantially free from tendency to flute or stretcher strain, which comprises cold rolling the sheet to gauge, annealing the same, treating the sheet to lessen its tendency to flute or stretcher strain, passing the same through a tin pot, and immediately thereafter, while still at an elevated temperature, reversely flexing the same and further reversely flexing the same while cooling.

HENRY W. NIEMAN.